

## UNITED STATES PATENT OFFICE.

BOHUMIL JIROTKA, OF BERLIN, GERMANY, ASSIGNOR TO THE FIRM DR. OTTO SPRENGER, PATENTVERWERTUNG JIROTKA MIT BESCHRANKTER HAFTUNG, OF VADUZ, LIECHTENSTEIN.

PROCESS FOR OBTAINING METAL COATINGS ON ARTICLES OF ALUMINUM AND ALUMINUM ALLOYS.

No Drawing. Application filed January 15, 1926, Serial No. 81,580, and in Germany October 29, 1924.

It is known to coat aluminum articles very thinly with copper, on which a thicker coating of nickel or the like can be electrical-  
ly deposited without the danger of the peeling-  
off which occurs when the nickel is  
deposited directly on to the aluminum. To effect such thin coating with copper the aluminum articles, after they have been sepa-  
rately freed from grease, are exposed to  
the action of a weak electric current in an  
acid bath of a copper salt.

In the art of coating metals it has also been proposed to coat aluminum with a preliminary layer of copper, zinc, or tin, by dipping in a solution of the fluoride of the coating metal and potassium tartrate. It has been further proposed to coat aluminum preliminarily with zinc by dipping the aluminum in sulphate of zinc and ammonium tartrate.

It has also been proposed to coat aluminum directly with a desired metal by dipping in a bath, which may be heated to hasten the action, composed of ammonium chloride and the chloride or the salt of the coating metal, the bath being rendered alkaline by the addition of liquid or aqua ammonia, or ammonium carbonate. A mixed coating may be obtained by using a suitable mixture of the salts of the coating metals.

According to the present invention a usable metal coating is obtained on aluminum both without preliminary freeing from grease and without employment of electric current by immersion in a bath of hot salt solution of alkaline reaction, which contains salts of copper, nickel, cobalt and zinc, manganese, iron and chromium, lead, bismuth, silver, gold and tin and in addition only potassium carbonate and potassium bicarbonate alone, or mixed with a corresponding salt or salts of sodium. Water-soluble oxygen liberating compounds in particular water-soluble chromate can be added to the bath.

A copper coating obtained in the presence of alkaline carbonate has a dark colour. A bright and clean metallic deposit is obtained if an oxidizing agent, in particular potassium bichromate, is added to the bath.

A bath which has proved extremely good in use contains in 2.5 litres of water 25 gms.

of crystalline copper sulphate, 25 gms. of potassium carbonate, 25 gms. of sodium bicarbonate and 10 gms. of potassium bichromate. Instead of 10 gms. of potassium bichromate up to 25 gms. of a 3% solution of hydrogen peroxide can be used. Instead of potassium carbonate and sodium bicarbonate a correspondingly greater quantity of potassium bicarbonate alone can be used.

In this bath the copper sulphate can be replaced by equivalent quantities of in-  
organic salts of heavy metals, so that a firmly  
adhering deposit can be obtained direct,  
that is without preliminary deposit of a  
layer of copper.

In this way it is possible by using the sulphate of nickel, cobalt, or manganese, iron, chromium, or zinc to produce firmly adher-  
ing metal coatings on aluminum. The same  
method succeeds with nitrates of lead, bis-  
muth or silver. The silver coating is at first  
bright, but with longer boiling takes on the  
dark colour, known as so-called oxidized  
silver.

By using tin chloride a coating of tin is also successfully obtained, which however does not have the bright appearance of the other coatings. By using gold chloride on the other hand a brilliant coating is obtained without the use of oxidizing agents.

The above mentioned metallic salts can also be used mixed to obtain mixed coatings. For example a mixed deposit of chromium and silver can be obtained on soft aluminum by using a solution containing in 1 litre of water, 10 gms. of chromium sulphate, 2 gms. of silver nitrate, 10 gms. of potassium carbonate, 3.3 gms. of sodium bicarbonate, and 3.3 gms. of potassium bichromate. For coating duralumin, three times the quantity of each constituent is used per litre. It has been found that the coatings are brighter if glycerine (e. g. 10-20%) is added to the metallizing baths.

Instead of articles of pure aluminum, those made of aluminum alloys, e. g. duralumin, can be coated.

It will be noted from the above descrip-  
tion that it is not necessary to use the  
poisonous cyanides or the expensive am-  
monia salts to produce a satisfactory coat-  
ing. In addition, as pointed out also in the

written description the process has the advantage that neither the electric current nor prior cleaning is necessary.

In certain of the claims the term "a substantial amount of" has been used before the name of certain ingredients or compounds. Such terms have been used to distinguish from cases in which mere traces of (or inconsequential amounts of) the said substances may possibly have been present as impurities in other substances used.

What I claim is:

1. The process for producing metal coating on aluminum or an aluminum alloy without substantial previous cleaning which comprises subjecting a surface thereof without application of electric current to the action of an aqueous liquid to which has been added a bicarbonate of an alkali metal and a simple salt of a metal which is electronegative to aluminum.

2. The process for producing metal coating on aluminum or an aluminum alloy which comprises subjecting a surface thereof to the action of an aqueous liquid to which has been added a bicarbonate of an alkali metal and a salt of a metal which is electronegative to aluminum.

3. The process for producing metal coating on aluminum or an aluminum alloy which comprises subjecting a surface thereof without application of electric current to the action of an aqueous liquid to which has been added an alkali carbonate, an alkali bicarbonate and a salt of a metal which is electronegative to aluminum.

4. The process for producing metal coating on aluminum or an aluminum alloy without substantial previous cleaning which comprises subjecting a surface thereof without application of electric current to the action of an aqueous liquid to which has been added bicarbonate of potassium and a simple salt of a metal which is electronegative to aluminum.

5. The process for producing metal coating on aluminum or an aluminum alloy which comprises subjecting a surface thereof to the action of an aqueous liquid containing potassium bicarbonate and a salt of a metal which is electronegative to aluminum.

6. The process for producing metal coating on aluminum or an aluminum alloy which comprises subjecting a surface thereof to the action of an aqueous liquid to which has been added a carbonate of an alkali metal, a substantial amount of bicarbonate of an alkali metal, at least one of said alkali metals being potassium, and a salt of a metal which is electronegative to aluminum.

7. The process for producing metal coating on aluminum or an aluminum alloy which comprises subjecting a surface thereof without application of electric current to the action of an aqueous liquid to which has been

added a bicarbonate of an alkali metal and a salt of a metal which is electronegative to aluminum.

8. The process for producing metal coating on aluminum or an aluminum alloy which comprises subjecting a surface thereof to the action of an aqueous liquid to which has been added a substantial amount of bicarbonate of an alkali metal, and oxygen liberating compound and a simple salt of a metal which is electronegative to aluminum.

9. The process for producing metal coating on aluminum or an aluminum alloy without substantial prior cleaning which comprises subjecting a surface thereof to the action of an aqueous liquid to which has been added a substantial amount of bicarbonate of potassium, an oxygen liberating agent, and salt of a metal which is electronegative to aluminum.

10. The process for producing metal coating on aluminum or an aluminum alloy which comprises subjecting a surface thereof to the action of an aqueous liquid to which has been added a substantial amount of potassium bicarbonate, an oxidizing agent and a salt of a metal which is electronegative to aluminum.

11. The process for producing metal coating on aluminum or an aluminum alloy which comprises subjecting a surface thereof to the action of an aqueous liquid to which has been added a carbonate of an alkali metal, a bicarbonate of an alkali metal, at least one of said alkali metals being potassium, an oxygen liberating compound, and a salt of a metal which is electronegative to aluminum.

12. The process for producing metal coating on aluminum or an aluminum alloy which comprises subjecting a surface thereof to the action of an aqueous liquid to which has been added a bicarbonate of an alkali metal, an oxygen liberating agent and a salt of a metal electronegative to aluminum.

13. The process for producing metal coating on aluminum or an aluminum alloy which comprises subjecting a surface thereof to the action of an aqueous liquid to which has been added a bicarbonate of an alkali metal, a carbonate of an alkali metal, an oxygen liberating compound and a salt of a metal which is electronegative to aluminum.

14. The process for producing metal coating on aluminum or an aluminum alloy which comprises subjecting the surface thereof to the action of an aqueous liquid to which has been added potassium bicarbonate, an oxidizing compound, glycerine and a salt of a metal which is electronegative to aluminum.

15. The process for producing metal coating on aluminum or an aluminum alloy which comprises subjecting a surface thereof

to the action of an aqueous liquid to which has been added a carbonate of an alkali metal, a bicarbonate of an alkali metal, at least one of said alkali metals being potassium, an oxygen liberating compound, glycerine, and a salt of a metal which is electronegative to aluminum.

16. The process for producing metal coating on aluminum or an aluminum alloy which comprises subjecting a surface thereof to the action of an aqueous liquid to which has been added a bicarbonate of an alkali metal, an oxygen liberating agent, glycerine, and salt of a metal which is electronegative to aluminum.

10 15

17. A bath mixture for coating aluminum or an aluminum alloy by contact with an aqueous mixture thereof containing a substantial amount of a bicarbonate of an alkali metal and a salt of a metal which is electro-negative to aluminum.

18. A bath mixture for coating aluminum or an aluminum alloy by contact with an aqueous mixture thereof containing a substantial amount of potassium bicarbonate and a salt of a metal which is electronegative to aluminum.

19. A bath mixture for coating aluminum or an aluminum alloy by contact with an aqueous mixture thereof containing an alkali carbonate, a substantial amount of an alkali bicarbonate and a salt of a metal which is electronegative to aluminum.

35 20. A bath mixture for coating aluminum or an aluminum alloy by contact with an aqueous mixture thereof containing a carbonate of an alkali metal, a substantial amount of a bicarbonate of an alkali metal, at least one of said alkali metals being potassium, and a salt of a metal which is electronegative to aluminum.

21. A bath mixture for coating aluminum or an aluminum alloy by contact with an aqueous mixture thereof containing a bicar-

bonate of an alkali metal, an oxygen liberating compound and a salt of a metal which is electronegative to aluminum. 45

22. A bath mixture for coating aluminum or an aluminum alloy by contact with an aqueous mixture thereof containing potassium bicarbonate, an oxygen liberating compound and a salt of a metal which is electronegative to aluminum. 50

23. A bath mixture for coating aluminum or an aluminum alloy by contact with an aqueous mixture thereof containing a substantial amount of potassium bicarbonate, an alkali chromate compound, and a salt of a metal which is electronegative to aluminum. 55

24. A bath mixture for coating aluminum or an aluminum alloy by contact with an aqueous mixture thereof containing a carbonate of an alkali metal, a substantial amount of bicarbonate of an alkali metal, at least one of said alkali metals being potassium, an oxygen liberating compound, and a salt of a metal which is electronegative to aluminum. 60 65

25. A bath mixture for coating aluminum or an aluminum alloy by contact with an aqueous mixture thereof containing a carbonate of an alkali metal, a substantial amount of bicarbonate of an alkali metal, at least one of said alkali metals being potassium, an alkali chromate compound, and a salt of a metal which is electronegative to aluminum. 70 75

26. A bath mixture for coating aluminum or an aluminum alloy by contact with an aqueous mixture thereof containing a carbonate of an alkali metal, a substantial amount of bicarbonate of an alkali metal, an oxygen liberating compound and a salt of a metal which is electronegative to aluminum. 80

In testimony whereof I affix my signature,

BOHUMIL JIROTKA